

June 28, 1938.

D. KLEIST ET AL.

2,121,802

## METHOD AND APPARATUS FOR STRENGTHENING FIBERS

Original Filed Aug. 30, 1935

FIG- 1 -



FIG-2 -



FIG-3 -



FIG-4-



Dale K. Kleist and  
John H. Thomas,  
INVENTORS

BY J. F. Rose, ATTORNEY.

## UNITED STATES PATENT OFFICE

2,121,802

METHOD AND APPARATUS FOR STRENGTH-  
ENING FIBERS

Dale Kleist and John H. Thomas, Newark, Ohio,  
assignors to Owens-Illinois Glass Company, a  
corporation of Ohio

Application August 30, 1935, Serial No. 38,568  
Renewed June 16, 1937

16 Claims. (Cl. 49—1)

Our invention relates to the production of fibers from molten or viscous materials and particularly to methods and means for subjecting the fibers during their formation, to vibratory forces by which their strength and elasticity are increased and the quality of the fibers materially improved.

The invention is herein particularly described and illustrated as used in the production of fibers from glass or other siliceous material. Such materials may be formed into fine fibers by flowing the molten material in small streams, and while the flowing material is cooling and in a viscous condition drawing it out into fine fibers or filaments which rapidly solidify or harden. We have discovered that by subjecting these fibers while in a viscous condition, and particularly while within an annealing temperature range, to sound vibrations or like periodic vibratory forces, the strength, elasticity and toughness of the fibers are materially increased and the quality of the fibers improved.

In practicing our invention, the flowing material which is being drawn into fibers is passed through a field of vibration while hot and in a plastic condition. It is believed that the vibratory forces acting on the viscous material cause molecular movement and adjustment as well as physical rearrangement of the material in a manner to produce the results above pointed out. The periodic or vibratory forces applied to the material may be either in the nature of sound vibrations, supersonic vibrations (above the range of audibility), or other forms of vibratory forces.

Referring to the accompanying drawing:

Fig. 1 is a sectional elevation of an apparatus adapted for practicing our invention.

Fig. 2 is a similar view showing a modification.

Fig. 3 is a similar view of a further modification.

Fig. 4 is a bottom sectional view, the section being taken at the line IV—IV on Fig. 3.

Referring particularly to Fig. 1, molten glass or other molten or viscous material is supplied to a refractory container 11 herein shown as a forehearth extension of a glass melting and refining tank 12. The glass flows in a small stream through an outlet opening 13.

Beneath the outlet is a blower 14 comprising a pressure chamber 15 to which steam or other gas under pressure is supplied. Extending through the blower is a central passageway 16 which is positioned beneath and in register with the outlet opening 13, permitting the stream 17 of viscous glass or the like to flow downward

therethrough. The blower is formed with an annular passageway or series of openings 18 through which steam or other gas is ejected from the pressure chamber. The blast of steam surrounds and envelops the stream 17.

The downwardly convergent blast impinges upon and grips the flowing stream and thereby continuously draws it out to the form of a fine filament which is carried downward at a high velocity by the steam blast. The flowing stream 10 is thus continuously attenuated to a fine fiber. This attenuation is produced by the force of the blast acting on the flowing material while the latter is in a viscous condition and while the material is cooling or passing through an annealing temperature range.

In accordance with our invention, the flowing material, while being thus attenuated, is subjected to vibratory forces, preferably in the form of sound or supersonic vibrations. One method 20 of producing effective vibrations of this character, consists in providing a tube or horn 20, beneath and cooperating with the blower 14. The tube is preferably made of sheet metal or other resonant material and is located directly 25 beneath and in register with the blower. As shown, the walls of this tube are downwardly and outwardly flared.

The steam under high pressure, issuing at high velocity through the outlets 18, sets up a rapid 30 vibration which may be manifested as a sound having a high pitch, or the vibrations may be above the range of audibility. The tube or horn 20 serves as an amplifier by which the force of the vibrations is greatly magnified. These vibrations impinging upon the flowing material while the latter is at an annealing temperature or within the working temperature range, cause a molecular and physical rearrangement and adjustment of the material in such a manner that the 40 resultant fiber has much greater strength and elasticity than it would have in the absence of such treatment.

Fig. 2 illustrates a modification in which the upper end of the horn 20 is spaced a short distance below the blower. This permits air to be drawn into the horn together with the descending blast of steam and results in a superior operation. The arrangement is also conducive to a stronger vibration of the horn, resulting in a 50 more effective action of the vibratory forces upon the flowing stream of glass. The blower as shown in Fig. 2, comprises a bushing 22 having a screw threaded connection with the body of the blower. This permits vertical adjustment of the bushing, 55

which results in adjusting the size of the outlet orifices through which the steam issues.

- Figs. 3 and 4 illustrate a modified design of blower which has been found very effective for the purposes of the present invention. The blower is formed with an annular series of small outlet openings 18' through which the steam issues in an annular series of downwardly convergent jets. These provide a steam blast of conical formation surrounding the stream of glass which enters the vortex of the blast and is gripped thereby and carried downward therewith at a high speed, thus attenuating the stream into a fine fiber.
- 15 The steam issuing through the multiplicity of small outlets 18' under high pressure, sets up a mechanical vibration which is transmitted to the flowing material through the surrounding gaseous medium. Such medium may consist of a 20 mixture or combination of the steam and the air which is drawn into and through the blower by the force of the steam.

The horn 20 is carried on a bracket 23 mounted for vertical adjustment on a stationary bracket 25 arm 24, being secured to the latter by clamping bolts 25 which extend through elongated slots 26 in the arm 24. The blower is secured by means of adjusting bolts 27 to a supporting plate 28 underlying the forehearth or container 11. This 30 construction permits vertical adjustment of the blower.

Modifications may be resorted to within the spirit and scope of our invention.

We claim:

35 1. The method which comprises flowing a molten stream of thermoplastic viscous material which forms a super-cooled solution at room temperature, applying a drawing force to the stream, by which it is attenuated, and applying to the 40 material while in a viscous state, a vibratory force.

2. The method of treating a molten inorganic thermoplastic material which is viscous at a high temperature and capable of rapidly passing from 45 a viscous to a hardened amorphous condition upon cooling, which comprises spinning the plastic material to the form of a fine fiber, rapidly cooling and hardening the material as it is formed into a fiber, and subjecting the fiber during formation and while the material is in a viscous or plastic condition, to a vibratory force effective to improve the quality of the fiber.

3. The method of treating a molten inorganic thermoplastic material which is viscous at a high 55 temperature and capable of rapidly passing from a viscous to a hardened amorphous condition upon cooling, which comprises spinning the plastic material to the form of a fine fiber, rapidly cooling and hardening the material as it is formed 60 into a fiber, and subjecting the fiber during formation and while the material is in a viscous or plastic condition, to sound vibrations effective to improve the quality of the fiber.

4. The method which comprises flowing a 65 stream of molten glass, subjecting the stream to a drawing force by which it is continuously drawn to the form of a fiber, and subjecting the glass during such formation and while in a viscous or plastic condition, to vibratory forces by 70 which the strength of the fiber is increased.

5. The method which comprises drawing a fiber from a supply body of molten glass, cooling the fiber as it is formed and causing the material to pass from a viscous to a solid or hardened condition, and applying sound vibrations to the fiber 75

during said cooling and thereby improving the quality of the fiber.

6. The method which comprises drawing a fiber from a supply body of molten glass, cooling the fiber as it is formed and causing the material to pass from a viscous to a solid or hardened condition, and subjecting the fiber during its transition from a plastic to a hardened condition, to supersonic vibrations by which the fiber is strengthened.

7. The combination of a container for molten glass provided with an outlet opening through which the glass issues in stream formation, and a blower by which the flowing glass is subjected to a blast of gas and continuously drawn to the 15 form of a fine fiber, said blower comprising a multiplicity of outlets or nozzles through which the gas under pressure issues, the blower being constructed to produce sound vibrations, and arranged to cause said vibrations to be impressed 20 upon the glass fiber.

8. The combination of a container for molten glass provided with an outlet opening through which the glass issues in stream formation, a blower by which the flowing glass is subjected to 25 a blast of gas and continuously drawn to the form of a fine fiber, said blower comprising a multiplicity of outlets or nozzles through which the gas under pressure issues, the blower being constructed to produce sound vibrations, and a resonator by 30 which the sound vibrations are strengthened, said parts arranged to apply the force of said sound vibrations to the forming filament and while the material is still plastic and thereby increase the strength and elasticity of the filament. 35

9. The combination of means for projecting glass in a viscous condition from a molten supply body, drawing the glass to fine fibrous form and causing it to cool and pass from a viscous to a solidified or hardened state during the drawing, 40 and means for subjecting the material to supersonic or sound vibrations while passing from a viscous to a hardened state.

10. The combination of means for projecting glass in a viscous condition from a molten supply body, drawing the glass to fine fibrous form and causing it to cool and pass from a viscous to a solidified or hardened state during the drawing, 45 and means for subjecting the material to supersonic or sound vibrations during said drawing operation.

11. The method of treating a thermoplastic material which assumes a viscous condition when at a high temperature and which solidifies or hardens into a super-cooled solution when cooled, 55 which method comprises drawing the hot viscous material to a fine filament, cooling and hardening the fiber, and subjecting the material during cooling to a periodic force of sufficient intensity to cause a molecular adjustment of the material 60 and thereby modify the characteristics of the hardened filament.

12. The method which comprises projecting hot viscous glass from a molten supply body and spinning it into fibers, subjecting the projected viscous glass to a cooling medium by which it is cooled and solidified, and applying to the fibers during solidification a periodic force of high frequency.

13. The method which comprises projecting 70 hot viscous glass from a molten supply body and spinning it into fibers, subjecting the projected viscous glass to a cooling medium by which it is cooled and solidified, and subjecting the fibers while in a viscous condition to a periodic force in 75

a direction transverse to that in which the fibers extend.

14. The method which comprises projecting hot viscous glass from a molten supply body and spinning it into fibers, subjecting the projected viscous glass to a cooling medium by which it is cooled and solidified, and subjecting the fibers during solidification to sound vibrations transmitted in a direction transverse to the fibers and acting on the fibers with sufficient force and intensity to modify the characteristics of the fibers.

15. The method which comprises flowing a stream of molten glass, applying to the stream a drawing force by which it is continuously attenuated and drawn to the form of a fine fiber, rapidly cooling the material during the drawing operation and thereby causing it to pass from a viscous to a solid condition during its attenuation, and subjecting the glass throughout the period of its

transition from molten stream form to a solid filament, to rapid vibratory forces by which the strength of the fiber is increased and its quality improved.

16. The method which comprises flowing a stream of molten glass, applying to the stream a drawing force by which it is continuously attenuated and drawn to the form of a fine fiber, rapidly cooling the material during the drawing operation and thereby causing it to pass from a viscous to a solid condition during its attenuation, and subjecting the glass throughout the period of its transition from molten stream form to a solid filament, to high frequency sound vibrations effective to improve the quality and increase the strength of the fiber.

DALE KLEIST.  
JOHN H. THOMAS.